

# UNITED STATES PATENT OFFICE.

LEWIS A. COLEMAN, OF NORFOLK, VIRGINIA, ASSIGNEE TO AMERICAN CHEMICAL & MANUFACTURING COMPANY, INC., OF NORFOLK, VIRGINIA, A CORPORATION OF VIRGINIA.

## OIL AND THE METHOD OF MAKING THE SAME.

1,223,150.

Specification of Letters Patent. Patented Apr. 17, 1917.

No Drawing.

Application filed March 27, 1915. Serial No. 17,392.

*To all whom it may concern:*

Be it known that I, LEWIS A. COLEMAN, a citizen of the United States, residing at Norfolk, in the county of Norfolk and State 5 of Virginia, have invented new and useful Improvements in Oil and the Method of Making the Same, of which the following is a specification.

This invention relates to an improved oil, and more particularly to an oil which possesses water-proofing characteristics and which will not harden or stiffen the surface to which the same is applied.

An object of this invention is to provide a composition of this character which will not stiffen the surface to which it is applied as, for instance, a fabric, which will support and fix a pigment to the surface to which the composition is applied, a composition which 20 when applied to leather will soften the same and make the leather water-proof, and a composition which carries a pigment and fixes the same to a wall when the composition is applied thereto and renders the wall 25 impervious to moisture.

The above objects and advantages of the invention are carried out in the improved composition which is here referred to as an oil, and which comprises an admixture of 30 the following ingredients:

|                                                                                                   |     |
|---------------------------------------------------------------------------------------------------|-----|
| Boiled or evaporated linseed oil                                                                  | 80% |
| Oil of eucalyptus                                                                                 | 10% |
| Spirits of turpentine or its described equivalent or varnish makers' and 35 paint makers' naphtha | 5%  |
| Resinous tar pitch                                                                                | 5%  |

Of the above ingredients, the linseed oil is first subjected to boiling whereby to extract or drive out the water contained therein. The oil of eucalyptus used is an extract from the eucalyptus tree, and is a recognized staple product readily obtainable. The spirits of turpentine is a distilled product of the pine tree, and the resinous tar pitch is the residue of spirits of turpentine during its process of manufacture.

The method of admixing the above-noted ingredients is as follows:

The linseed oil after having the water extracted therefrom is again heated to the boiling point. The resinous tar pitch is reduced to a perfectly melted state by heating. The

spirits of turpentine and the oil of eucalyptus are commingled into one mixture. 55

Preferably, two tightly covered boilers connected by a pipe are used, the lower boiler containing the linseed oil and the upper boiler containing the resinous tar pitch. The linseed oil in the lower boiler 60 is maintained at the boiling point, and the resinous tar pitch in the upper boiler is permitted to flow gradually into the lower boiler to admix with the boiling linseed oil. This mixture is maintained at the boiling 65 point until the combined spirits of turpentine and oil of eucalyptus have been added thereto. This new composition becomes a heavy bodied mixture and may be diluted to any desired strength by adding thereto 70 varnish makers' and paint makers' naphtha and tri-chlorethylene.

It is, of course, understood that the proportions above given may be slightly varied for the application of the composition to 75 various surfaces and materials.

What I claim is,—

1. An oil comprising a mixture of evaporated linseed oil, oil of eucalyptus, spirits of turpentine, and resinous tar pitch, in substantially the proportions stated. 80

2. An oil comprising substantially evaporated linseed oil 80%, oil of eucalyptus 10%, spirits of turpentine or its described equivalent 5%, and resinous tar pitch 5%. 85

3. An oil comprising a mixture of linseed oil, oil of eucalyptus, spirits of turpentine, varnish makers' and paint makers' naphtha, and resinous tar pitch in substantially the proportions stated. 90

4. An oil comprising an admixture of evaporated linseed oil, oil of eucalyptus, spirits of turpentine or its described equivalent, resinous tar pitch, and tri-chlorethylene in substantially the proportions stated. 95

5. An oil comprising an admixture of evaporated linseed oil, oil of eucalyptus, spirits of turpentine, resinous tar pitch, and a diluent in substantially the proportions stated. 100

6. The process of making the herein-described oil which consists in extracting water from linseed oil and then heating the same to boiling point, heating resinous tar pitch to reduce the same to a melted state 105 and gradually mixing the pitch with the

boiling linseed oil, mixing spirits of turpentine and oil of eucalyptus into one mixture and then adding the mixture of spirits of turpentine and oil of eucalyptus to the mixture of boiling linseed oil and resinous tar pitch.

In testimony whereof I have hereunto set

my hand in presence of two subscribing witnesses.

LEWIS A. COLEMAN.

Witnesses:

JONATHAN W. OLD, Jr.,  
JOHN W. DASTZ.